

Feb. 15, 1938.

G. KAUFMAN

2,108,672

GREASE MANUFACTURE

Filed June 7, 1935



Gus Kaufman  
INVENTOR

BY *R. J. Dearborn*

his ATTORNEY

## UNITED STATES PATENT OFFICE

2,108,672

## GREASE MANUFACTURE

Gus Kaufman, Beacon, N. Y., assignor to The  
Texas Company, New York, N. Y., a corpora-  
tion of Delaware

Application June 7, 1935, Serial No. 25,361

3 Claims. (CL. 87-9)

This invention relates to the manufacture of grease.

An object of the present invention is to increase the hardness of a soda base grease without increase in the soap content thereof.

It has heretofore been suggested to pass grease through a milling machine of the character of a burr stone mill, to work down or reduce the hardness of the grease and minimize lumpiness.

As distinguished from the working down or reduction in hardness resulting from passing grease through such a burr stone mill, I have discovered that when greases of the soda base type are passed through a colloid mill, a definite increase in hardness of the grease results, which is the opposite of what would be expected.

In accordance with the present invention, a soda base grease is passed in a thin film between highly rotating closely spaced surfaces where it is thrown outwardly by centrifugal force while being subjected to a powerful shearing action, to thereby give a substantial increase in hardness of the grease, generally expressed as a decrease in consistency or a reduction in A. S. T. M. penetration of the grease. This is preferably accomplished by passing the grease between oppositely rotating discs of a colloid mill. Any suitable type of conventional colloid mill of this character may be employed. The grease may be heated to render it sufficiently fluid for pumping, and is passed in heated condition through the mill. Ordinarily, a single passage through a high speed colloid mill having discs rotating in opposite directions at a speed of around 2000-5000 R. P. M., will give a very substantial decrease in A. S. T. M. penetration. If desired, the grease can be recirculated through the mill until a desired penetration is obtained. As a result of this procedure, greases can be made of specified consistencies with lower soap content, thereby reducing the cost as a result of substituting the cheaper mineral oil constituent for the more expensive soap constituent. In addition, this procedure insures the elimination of soap lumps and gives a more uniform product.

Referring to the attached drawing, which illustrates a preferred embodiment of apparatus for practicing the method of this invention, a suitable soda base grease is maintained in a heated condition in vat 10 provided with steam jacket 11. The grease, which is sufficiently fluid for pumping, is withdrawn from vat 10 through line 12 by charge pump 13 and delivered through line 14, hollow shaft 15 and a centrally arranged opening in disc 16 of a colloid mill. Line 14 is connected with the rotary hollow shaft 15 by a suitable coupling and stuffing box 18.

The type of colloid mill illustrated is that known as the U. S. colloid mill, although any suitable conventional mill of this character can be em-

ployed. This mill comprises two oppositely rotating discs 16 and 20, mounted on shafts 15 and 21 respectively, which are positively driven in opposite directions by motors 22 and 23 respectively, through shafts 22' and 23' and gearing 5 24 and 25. The discs are enclosed within a suitable casing 26. Peripheral edges of discs 16 and 20 are set very close together by proper adjustment of shaft 21 by means of screw 21', so that the grease is subjected to a high shearing force 10 as it is thrown outwardly between the discs by centrifugal force.

The grease discharged from the peripheries of the discs is caught within casing 26, from where it is discharged by pipe 27 into reservoir 28. In 15 case it is desired to pass the grease a plural number of times through the mill, this may be accomplished by recirculating the grease from the reservoir 28 through line 29 by pump 30, which 20 delivers it through line 31 to the vat 10.

As a specific example, a U. S. colloid mill equipped with two steel discs of 6" diameter each, and driven in opposite directions by 3 H. P. motors at 3500 R. P. M., was employed. A soda base grease of the type adapted for automotive 25 lubrication, and having the following approximate composition:

|                                             | Percent |
|---------------------------------------------|---------|
| Cylinder stock (S. U. vis. 185-195/210° F.) | 95.5    |
| Sodium soap of hard tallow                  | 4.0     |
| Water                                       | 0.5     |

was passed once through the above colloid mill. The grease had an initial A. S. T. M. penetration of 438, while after treatment the A. S. T. M. penetration was 352.

A similar type of soda base grease having the following approximate composition:

|                                             | Percent |
|---------------------------------------------|---------|
| Cylinder stock (S. U. vis. 160-170/210° F.) | 89.5    |
| Sodium soap of hard tallow                  | 10.0    |
| Water                                       | 0.5     |

was reduced from an initial A. S. T. M. penetration of 340 to an A. S. T. M. penetration of 238 by one through passage in the above mill.

A soda base grease of the type of a sponge grease adapted for use on shaft bearings, and having the following approximate composition:

|                                                             | Percent |
|-------------------------------------------------------------|---------|
| Distillate mineral lubricating oil (S. U. vis. 180/100° F.) | 84.5    |
| Sodium soap of hard tallow                                  | 14.0    |
| Water                                                       | 1.5     |

was reduced in penetration (A. S. T. M.) from 55 280 to 229 by a single passage through the above mentioned mill.

Obviously, many modifications and variations of the invention, as hereinbefore set forth, may be made without departing from the spirit and 60

scope thereof, and therefore only such limitations should be imposed as are indicated in the appended claims.

I claim:

- 5 1. The method of increasing the hardness of a soda base grease of fibrous texture and water content not substantially in excess of about 1.5%, without increasing the soap content, which comprises, after completing the operations of saponifying the fat and mixing with mineral oil to form a homogeneous grease, heating the homogeneous 5 grease until fluid, pumping the fluid grease in a thin film through closely spaced positively driven high speed oppositely rotating smooth surfaces where it is thrown outwardly by centrifugal force while being subjected to a shearing action, with 10 resultant substantial decrease in the A. S. T. M. penetration of the grease, and then passing the grease without further treatment to a zone of collection for packaging for use.
- 10 15 2. The method of increasing the hardness of a soda base grease of fibrous texture and water

content not substantially in excess of about 1.5%, without increasing the soap content, which comprises, after completing the operations of saponifying the fat and mixing with mineral oil to form a homogeneous grease, heating the homogeneous 5 grease until fluid, pumping the fluid grease in a thin film through closely spaced positively driven high speed oppositely rotating smooth surfaces where it is thrown outwardly by centrifugal force while being subjected to a shearing action, with 10 resultant substantial decrease in the A. S. T. M. penetration of the grease, and then passing the grease without further treatment to a zone of collection for packaging for use.

3. The method of claim 2, in which the grease 15 is recirculated from the zone of collection back to the heating zone and then through the rotat-ing surfaces until a desired decrease in A. S. T. M. penetration is obtained.

GUS KAUFMAN. 20